

Patented July 23, 1929.

1,721,768

# UNITED STATES PATENT OFFICE.

EDWARD C. BURDICK, OF MIDLAND, MICHIGAN, ASSIGNOR TO THE DOW CHEMICAL COMPANY, OF MIDLAND, MICHIGAN, A CORPORATION OF MICHIGAN.

## MAGNESIUM ALLOY AND METHOD OF MAKING SAME.

No Drawing.

Application filed December 9, 1924. Serial No. 754,856.

The difficulties involved in alloying copper and manganese with magnesium will be found set forth in U. S. Patent No. 1,334,193 issued to W. R. Veazey, March 16, 1920. According to the method disclosed in this patent the desired amount of copper is first inter-fused with the magnesium and then the desired amount of manganese added in the form of anhydrous manganese chloride to the copper-magnesium alloy that is thus preliminarily formed. The manganese chloride is reduced to the metal by the excess of magnesium present, as explained in Patent No. 1,377,374 issued to W. R. Veazey, May 10, 1921.

I have discovered that the alloy containing the three metals in question, in which magnesium is the predominant constituent, may be more conveniently made by first alloying together the manganese and copper and then adding this preliminarily formed alloy to the magnesium. In fact, an alloy of the two first named metals is already known under the name of cupro-manganese, which ordinarily contains 70 per cent of copper and 30 per cent of manganese, and by adding the proper amount of this alloy to a given weight of magnesium the ternary alloy may be readily made, although such alloy will of course be limited, except as other additions be made thereto, to the same relative proportions of copper and manganese as are found in such cupro manganese. However, a ternary alloy of this composition has been found to possess several desirable characteristics.

The invention then consists of the new product, viz, an alloy containing magnesium in predominant amount and a relatively small amount of copper and manganese in approximately the proportions stated, together with the several steps involved in the making of such alloy hereinafter fully described and particularly set forth in the claims.

The following description it will be understood thus sets forth but one of the several ways in which the invention may be carried out.

The manner in which cupro manganese is made, this being a well known alloy, need not be described herein, it being sufficient to note that the standard composition of this alloy is, as stated above, 70 per cent copper and 30 per cent manganese. In utilizing this ready to hand material for the making of the desired ternary alloy, in which mag-

nesium is the predominant ingredient i. e. is present in substantial excess of one half the total, I first melt a measured quantity of magnesium in a suitable crucible or melting pot, preferably using a flux of slightly greater specific gravity than the molten metal and having sufficient surface tension to cause it to form a film thereover and thus prevent exposure of the metal to the atmosphere. The cupro manganese is then added to such molten magnesium, dissolving completely and fairly promptly, thorough intermixture being insured by stirring if necessary.

The molten alloy may then be conveniently removed from the crucible or melting pot by means of an ordinary ladle and is cast into bars or such other shapes as may be desired. While the amount of cupro manganese thus added may be varied, I have found very satisfactory results are obtained where it is added in an amount equal to one per cent of the total mass. This will give a resulting alloy in which the copper and manganese will aggregate approximately one per cent of the total, being actually slightly less due to losses inherent in the process. The proportion of the copper to the manganese will, however, remain substantially unchanged.

Thus, for example, 20 pounds of magnesium may be melted up and 90 grams of cupro manganese added, such addition being calculated to give an analysis of 0.70 per cent copper, and 0.30 per cent of manganese. The actual analysis of the resultant ternary alloy then shows approximately 0.70 per cent of copper and approximately 0.20 per cent of manganese, indicating that not all of the manganese has remained in the final alloy. I have been able to obtain by the foregoing method a manganese content as high as 0.26 per cent of manganese.

Castings made from the resultant alloy have a very fine grained structure even when the metal is poured very hot in casting. This is a consequential advantage, since with many magnesium alloys the proper pouring temperature has to be ascertained and carefully observed. Test bars made from an alloy having the composition first given above show an average yield point of 8240 pounds, and an ultimate strength of 20,200 pounds.

It will be understood that while I have specifically described the addition of cupro-manganese to magnesium alone, it may be

added to other alloys of the general type in which magnesium predominates, i. e. largely exceeds one-half of the total. Thus such cupro-manganese may be added to the known 5 alloy of magnesium with aluminum (see United States patent to Pistor, et al. No. 950,290) containing the last named metal in various amounts up to 20 per cent, the specific 10 illustration given containing 92 per cent magnesium and 8 per cent aluminum.

Other modes of applying the principle of my invention may be employed instead of the one explained, change being made as regards the composition and method herein disclosed, 15 provided the ingredients or steps stated by any of the following claims or the equivalent of such stated ingredients or steps be employed.

I therefore particularly point out and distinctly claim as my invention:—

1. The method of making a copper-man-

ganese-magnesium alloy, which consists in interfusing with magnesium a relatively small amount of cupro-manganese having the copper and manganese present in approximately 25 the ratio of seven to three.

2. The method of making a copper-manganese-magnesium alloy, which consists in melting a quantity of magnesium, and then adding thereto approximately one per cent 30 of cupro-manganese.

3. The method of making a copper-manganese-magnesium alloy, which consists in melting a quantity of magnesium, and then adding thereto approximately one per cent 35 of cupro-manganese wherein the copper and manganese are present in approximately the ratio of seven to three.

Signed by me this 5th day of December, 1924.

EDWARD C. BURDICK.